

Dec. 31, 1968

P. V. CATLOS

3,418,799

TWINE

Filed Jan. 28, 1965

FIG. 1.



FIG. 2.



INVENTOR

Peter V. Catlos

BY

Lawrence I. Freed

ATTORNEY

**1**

3,418,799  
TWINE

Peter V. Catlos, Montreal, Quebec, Canada, assignor to  
Cordex Limited, Ottawa, Ontario, Canada  
Filed Jan. 28, 1965, Ser. No. 428,880  
Claims priority, application Canada, Jan. 31, 1964,  
894,553  
7 Claims. (Cl. 57—152)

**ABSTRACT OF THE DISCLOSURE**

This invention is a binder twine comprising a resilient core consisting of continuous filament, twisted or un-twisted strands of viscose, polypropylene or nylon or other resilient synthetic filament, and a cover or wrapping consisting of extensible paper, such as kraft paper, twisted about the core.

This invention relates to a twine and in particular to a binder twine formed from a resilient, synthetic filament core and an extensible cover formed of a suitable paper such as kraft.

Many different types of twine for binders and other uses are presently known. Such twines are generally formed from natural fibers such as manila, jute, cotton, hemp and sisal fibers, kraft paper and the like. In some instances these materials are used alone whereas in other instances as exemplified by U.S. Patent No. 1,320,920, issued on Nov. 4, 1919 to G. L. Rice, the fibers are wrapped in a paper covering. Few if any advantages are obtained by wrapping natural fibers in paper and consequently the increased cost of such a twine is not justified.

Another known type of twine is the combination of kraft paper and fiber glass disclosed in U.S. Patent No. 2,861,416, issued to American Sisalkraft Corporation on Nov. 25, 1958.

Twine utilizing fiber glass may be quite strong but is also relatively stiff and when placed under tension is of limited extensibility. Furthermore such a twine is inclined to be brittle, hard on the hands when hand tying, and not particularly suitable for use in binders. Also use as twine of other synthetic filaments by themselves has been suggested. Various disadvantages such as lack of the bulk required for binders, lack of wet strength, and lack of knot holding ability are attendant upon such use.

Alternatively fiber glass may be used as a core material in a twine and a kraft paper cover wound about it but this type of twine is also stiff and since the extensibility of the core is substantially less than the cover, the fiber glass core will break at the limit of its extensibility without necessarily breaking the cover thus rendering the twine useless without being visibly so.

The present invention provides a twine particularly suitable for use in binders and which can be readily knotted, with conventional machinery; possesses satisfactory stretch, strength and flexibility and otherwise meets the requirements for a satisfactory replacement for sisal binder twine. The twine of this invention consists of two components both of which are extensible and under tension have substantially the same breaking point. Thus when the twine of the present invention is placed under stress the core material and cover material, while having two separate breaking points, have breaking points which are close enough together that they appear to break simultaneously. This characteristic results in good knotting ability.

Furthermore, depending upon the embodiment utilized

5

**2**

the twine of this invention will be found quite water resistant and rodent resistant, a feature of significance when used as binder twine. Also, the twine of this invention has been found to possess an improved weight/strength ratio and will normally perform much better than equivalent natural fiber twine in this regard as it will have approximately half the weight and three times the tensile strength of the equivalent natural cordage.

The invention will be better understood from the single sheet of drawings accompanying this application in which

FIGURE 1 is a plane view schematically showing the preparation of the twine, and

FIGURE 2 is a section through plane 2—2 of FIGURE 1.

The twine of the present invention is made with a core consisting of continuous filament, twisted or un-twisted strands of any of viscose, polypropylene or nylon, and a cover consisting of extensible paper such as kraft twisted about the core. If un-twisted filaments are employed they usually become twisted when the cover is wrapped about the core. Depending upon requirements, normal or wet strength paper may be used.

To form the twine of this invention suitable paper such as kraft paper sold under the name Clupack is cut in long strips of a suitable width depending upon the diameter of the core material. Clupack is a kraft paper which has been microscopically crimped across its direction of run in order to make it extensible in one direction.

Before twisting the paper about the synthetic filament core its is passed through a water bath at room temperature with any one portion of the paper remaining in the bath for a period of time sufficient to saturate it. In the situation where a paper possessing low wet strength is used, it should be soaked in mineral oil rather than water before twisting about the core.

The purpose of impregnating the paper in this manner is to make it sufficiently pliable for twisting and also depending upon the contents of the bath, the paper so impregnated will affect the stiffness or softness of the twine produced and thus this characteristic can be controlled to some extent.

The following three solutions for treating kraft paper possessing wet strength can be utilized, these being listed in order of the degree of pliability they impact to the paper, the last noted solution providing the greatest pliability.

(1) Water having a pH of about 7 and a hardness factor of 3—9 grains. In addition to magnesium and/or calcium salts other minerals commonly found in hard water may be present.

(2) One and one-half gallons of a wax emulsion sold under the trademark Nopco 2252-P by Nopco Chemical Co. Ltd., and one and one-half gallons of sulphonated castor oil sold under the trademark Monosul PH by Nopco Chemical Co. Ltd., mixed in one hundred gallons of soft water having a pH of about 7 to 12.

(3) Three gallons of the above-noted wax emulsion and three gallons of the above-noted sulphonated castor oil mixed in one hundred gallons of soft water having a pH of 7 to 12.

After being passed through the bath the strip of kraft paper is twisted about the core material by means of a standard ring or cube twister and the resulting twine is wound on a twister spool and permitted to dry after which it can be used in any binder or in other forms of wrapping and tying machines.

I claim:

1. A twine comprising a core of extensible synthetic

plastic filaments and an extensible paper cover wound about said core.

2. A twine comprising a core of extensible polypropylene filaments and an extensible kraft paper cover wound about said core.

3. A twine comprising a core of extensible viscose filaments and an extensible kraft paper cover wound about said core.

4. A twine comprising a core of extensible nylon filaments and an extensible kraft paper cover wound about said core.

5. The twine of claim 1 wherein the kraft paper is used.

6. The twine of claim 5 wherein said paper is of the type which has been microscopically crimped across its direction of run to render it extensible.

7. The twine of claim 1 wherein the paper is of high wet strength.

## References Cited

## UNITED STATES PATENTS

|   |           |         |                |         |    |
|---|-----------|---------|----------------|---------|----|
| 5 | 1,376,618 | 5/1921  | Hansen         | 139—420 | XR |
|   | 1,764,524 | 6/1930  | Reber          | 57—151  | XR |
|   | 2,128,302 | 8/1938  | Katz           | 57—150  |    |
|   | 2,388,745 | 11/1945 | Katz           | 57—151  | XR |
|   | 2,832,190 | 4/1958  | Bacon          | 57—140  | XR |
|   | 2,901,005 | 8/1959  | Schwartz       | 57—140  | XR |
|   | 3,126,699 | 3/1964  | Lefevre et al. | 57—167  | XR |
|   | 3,282,038 | 11/1966 | Howell         | 57—167  | XR |
|   | 2,465,081 | 3/1949  | Fleischer      | 87—6    |    |

15 FRANK J. COHEN, *Primary Examiner*.

DONALD E. WATKINS, *Assistant Examiner*.

U.S. Cl. X.R.

57—151